

Jan. 26, 1932.

E. CUMBERLAND

1,842,541

METHOD OF AND MEANS FOR THE PREVENTION OF CORROSION

Filed March 12, 1927



Fig. 1.



Fig. 2.



INVENTOR

Elliott Cumberland

BY Darby & Darby

his ATTORNEYS

## UNITED STATES PATENT OFFICE

ELLIOTT CUMBERLAND, OF KINGSTON HILL, ENGLAND

## METHOD OF AND MEANS FOR THE PREVENTION OF CORROSION

Application filed March 12, 1927, Serial No. 174,905, and in Great Britain June 15, 1926.

The general object of this invention relates to an improved method of and means for the prevention of corrosion in metals or metallic articles which are, or are liable to be immersed in, or in contact with liquids capable of acting as electrolytes.

It is well known that where an electrolyte is in contact with two different metals galvanic action may occur which results in corrosion, and the prevention of corrosion for example of ships' hulls, stern frames, propellers, boilers, condensers and the like, both of the marine and land types, has long been a difficult problem. It has been generally supposed that this corrosion was due entirely to electro-chemical or galvanic action, such for example as that which occurs between a bronze propeller and the steel hull of a ship with the sea as an electrolyte, or to differences of temperature causing thermo-galvanic pairs, which may occur in boilers, condensers and the like.

In order to prevent this type of corrosion, I have previously proposed to employ a separate source of electrical energy, such as a dynamo and to connect the positive pole thereof to insulated anodes in the various boilers, condensers, stern frames and the like to be protected whilst the negative pole is connected to the hull of the ship or to the actual part that is to be protected.

It was found that where the corrosion was due entirely to causes of the kind referred to this method gave satisfactory preventive results but in some cases which for a long time were difficult to explain the method was found to be unsuccessful.

As a result of prolonged experiment I have now found that in addition to the causes referred to such as ordinary galvanic or electro-chemical action, corrosion of metals is frequently due to electro-disturbances or stray currents, leaks or the like, resulting from the operation of electric or other machinery.

As instances of such causes I may mention by way of example only that in the case of ships, corrosion has been found to be due to leakage from electric plant such for example as a lighting and power set. Moreover it has

been found both in the case of marine and land turbines that stray currents generally of very high potential are set up, the cause in some cases being the impinging of the steam on the turbine blades and such stray currents have also been found to cause corrosion.

It has also been found that in many instances metallic substances such for example as water mains, have been corroded unduly, rapidly in the vicinity of electric generating stations and I have found that such corrosion is again due to stray currents or leakages from the electric plant.

Now the method above described has been found to be unable to protect metallic articles from corrosion due to any of the latter type of causes and according to the present invention I provide an improved method of and means for protecting metallic substances against corrosion due to causes of this type.

According to the invention therefore I protect metallic articles from corrosion due to causes of the kind referred to by arranging for all the actual source of corrosion producing electric currents or disturbance to be so connected to the article or articles to be protected that the latter form part of the negative end of the circuit.

In other words I have found that the provision of a separate source of electrical energy for rendering the articles to be protected negative is not capable of producing the desired effect but that the protection can only be afforded by the combined effects of all the sources of energy which would otherwise cause the corrosion.

Preferred methods of carrying out my invention as applied to certain specific devices or structures, will now be described by way of example only, and are illustrated in the accompanying drawings in which:

Fig. 1 shows in part sectional elevation how the invention can be applied to water mains, and

Fig. 2 a diagrammatic plan view of the application to a marine turbine and condenser plant.

Referring to Fig. 1 which shows the application of my invention to a water main in the vicinity of say an electrical generating sta-

tion, within the main 1 is housed an insulated anode bar 2 suitably supported as by insulating members 3 and having electrical connection with terminals 4 to which leads 17, 18 and 21 are taken from the positive pole of the generators 15 and 19, the main 1 being similarly connected to their negative poles by wires 16 and 22. Internal corrosion caused by stray currents passing through the fluid within the main is thus prevented and in order to prevent external corrosion from the same causes, and in which the damp earth may act substantially as an electrolyte, an anode bar 5 is buried in close proximity to the part of the main where corrosion is taking place and has the positive potential of the generator impressed thereon in a similar manner to that in the case of the internal anode.

As remarked generally below resistances may be used in the leads of the generators, especially when several are used in order that the currents passing to the electrodes of the articles to be protected may be properly adjusted to effectively prevent corrosion. As shown in Fig. 1 the negative lead includes the variable resistance 100 and the positive lead includes the variable resistance 101. The main lighting or power circuit wires leading from the generators are indicated at 50 and 51. As illustrated in Fig. 1, if the leak should occur at X in the positive leg 50 of the main circuit, current would flow through any conducting path passing from the leak to the article 1 to be protected, and through the wall of the article to the negative connection and back to the generator. Should a leak occur in the negative leg of the circuit no current will flow, since the objects are then connected to the negative side of the current source and not through the conducting medium around, and in the article are maintained at the proper positive potential by means of the electrodes 2 and 5. As a result, when the resistances 100 and 101 are properly adjusted no stray currents can leave the articles to be protected in the direction to effect corrosion thereof at the points where currents would otherwise lead.

It will be apparent that the method described can be applied for protecting mains externally, internally, or for both purposes.

Figure 2 shows in diagrammatic plan view the application of my invention to the protection of a condenser 9 from corrosion caused by stray currents from a marine turbine shown at 11, such currents being caused in some cases by steam issuing at high velocity from the turbine nozzles and impinging on the blades causing a difference of potential to be set up, the oil between the rotor shaft and its bearing acting as an insulator between said rotor and the stationary part of the turbine structure. In this case I provide copper gauze or other suitable brushes 6 either di-

rectly in contact with the shaft 7 or in contact with collector rings shown at 12 carried thereon and having electrical connection with anodes 8 supported on insulating members 13 wholly or partially submerged within the electrolyte in the condenser 9, the condenser body itself being maintained at negative potential by connection 14 with the turbine casing, alternatively electrical connection may be made between the turbine shaft and the casing or otherwise earthing the lead therefrom. In the case of a ship's lighting and power dynamo being the cause of corrosion I run leads if necessary through one or more suitable resistances from the positive pole of said dynamo to the anodes and from the negative pole to the article to be protected.

I have found that in many cases the method herein described will act as a protection against corrosion caused by ordinary electrochemical or galvanic action and in some cases this has even been found to be successful where the corrosion producing source of electrical energy has only been intermittently in operation, such for example as in the case of a ship's lighting set. This is probably due to the negative polarisation of the article to be protected and the formation of a film of hydrogen thereon which effects have lasted until the set has again been put into operation. It should, however, be noted that where necessary or desirable the present invention may be applied together with previously known protective methods involving the use of separate sources of electrical energy.

This invention may generally be applied to all metallic structures or the like which are or which are liable to be subjected to corrosive action of the types referred to, and which are liable to be immersed in or in contact with liquids capable of acting as electrolytes. Among such articles I may mention for example bridges, reinforced ferro-concrete buildings, fluid conduits, floating docks, gasometers, piers and lock gates in addition to those examples already given.

In the foregoing I have described by way of example several methods of carrying out my invention but it will be apparent that these can be varied within wide limits without departing from the scope thereof, the essential feature in each case being that the same source or sources of electrical energy which is or are causing the corrosion are utilized to prevent it by rendering the article or articles to be protected negative to the particular source or sources of electrical energy in question, a corresponding positive pole or plurality thereof being insulated from said article or articles and immersed or partially immersed, in the electrolyte so that current can only flow through such electrolyte in the desired direction.

I claim:

1. The method of preventing the destruc-

tion of metallic objects in contact with an electrolyte by electrolytic decomposition by electric currents from a current source comprising connecting the negative side of said current source to the object to be protected, providing an electrode adjacent the object to be protected and connecting the electrode to the positive side of said current source.

2. The method of preventing the destruction of hollow metallic objects by electrolytic decomposition by electric currents from a current source comprising connecting the negative side of said current source to the object to be protected and connecting the positive side of said current source to electrodes inside of and outside of the object to be protected.

3. In an arrangement as described, the combination with a current source of a metallic object to be protected from electrolytic decomposition, said object being in contact with an electrolyte, a connection between the negative side of said current source and said metallic object, an electrode in contact with the electrolyte and a connection between the positive side of said current source and said electrode.

4. In an arrangement as described, the combination with a current source of a hollow metallic object to be protected from electrolytic decomposition, said object surrounding an electrolyte and in contact with it, a connection from the negative side of said current source to said object, an electrode supported within said object and insulated therefrom and in contact with the electrolyte, another electrode in contact with the electrolyte and connections from the positive side of said current source to said electrodes.

5. In an arrangement as described, a metallic object in contact with a conducting medium, current sources in electrical contact with the electrolyte, a connection from the negative side of each of said sources to said metallic object, an electrode in contact with the electrolyte and a connection from the positive side of each of said current sources to said electrode.

6. The method of preventing the destruction of metallic objects in contact with an electrolyte by electrolytic decomposition by electric currents from current sources, comprising ascertaining all of the sources of the corrosion producing currents, connecting all of the negative sides thereof to the article to be protected, providing electrodes adjacent the object to be protected and connecting all of the positive sides of the corrosion producing sources to said electrodes.

7. In testimony whereof I have hereunto set my hand this 25th day of February, 1927.

ELLIOTT CUMBERLAND.